

Oct. 21, 1947.

A. M. COHAN

2,429,548

PROPELLENT FUEL CARTRIDGE

Filed Sept. 20, 1943



Alvin M. Cohan  
INVENTOR

BY *Kenneth E. Mulford*  
ATTORNEY

## UNITED STATES PATENT OFFICE

2,429,548

## PROPELLENT FUEL CARTRIDGE

Alvin M. Cohan, North Bergen, N. J., assignor to  
 Atlas Powder Company, Wilmington, Del., a  
 corporation of Delaware

Application September 20, 1943, Serial No. 503,095

2 Claims. (Cl. 102—39)

1

The present application relates to propellant fuel cartridges.

An object of the present invention is to prepare an improved propellant fuel cartridge, and particularly a cartridge of superior design which is adapted to perform useful mechanical work as in a prime mover, such as an engine starting mechanism.

It is a further object of the present invention to provide a cartridge which will avoid the necessity for using special ignition receiving fuels, such as double base smokeless powder.

It is another object of the invention to provide improved resistance to quenching in a propellant fuel cartridge.

A still further object of the invention is to provide a cartridge which will permit the use of simplified fuel charges without loss of efficiency.

Other objects of the invention will appear from the following description.

For a number of years cartridges containing propellant fuel have been employed to do mechanical work, often through the medium of a piston on which expanding burning gases from the fuel may work. Such cartridges have found special utility for use in supplying power for starters for internal combustion engines.

Propellant fuel cartridges which are to be used to supply power to actuate a prime mover or otherwise supply useful power should rapidly, but not explosively, produce a large volume of gas capable of doing work. If gas pressure is produced too slowly, efficiency is lost through excessive heat losses to cold mechanical equipment, while if gas pressure is produced explosively, it may break the mechanical equipment before useful work can be done. Smokeless powder (colloided nitrocellulose) has been found most satisfactory for use as a fuel in cartridges of the present type. This fuel has, however, been difficult to ignite and burn efficiently and completely under the conditions of low confinement usually obtaining in power producing systems such as engine starters. The sudden gas expansion apparently interferes with the complete ignition of the fuel. A number of expedients have been employed to improve the burning characteristics of propellant fuel cartridges. Usually, for best results, it has been found necessary to include some double base powder (colloided nitrocellulose plus nitroglycerine). Also it has been found necessary to load cartridges with a succession of different sized fuel particles. A further expedient which has been employed has been to carry a column of flash composition from the igniting means (which usually lies at the base of the cartridge) up to the front end of the cartridge so as to ignite the cartridge shell from both ends. All of these methods of improving the burning characteristics of cartridges have

some disadvantages. The use of double base powders is considered to be objectionable for cartridges used under some circumstances. The loading of different sized fuel particles, deck loading as it is called, is unduly expensive and troublesome, as is also the expedient of carrying the column of flash composition from the back to the front end of the cartridges.

Also cartridges of the prior art have not proven as consistent as desirable when a number are used in succession in the same apparatus. Particularly is this true when low ambient temperatures prevail. Under such conditions, the cartridges tend to quench out before complete combustion takes place.

It has been found, according to the present invention, that cartridges may be prepared which need contain no double base powders and which may contain a single size powder, and yet be entirely satisfactory as to power produced and resistance to quenching.

Such cartridges are prepared by coating the inside surface of the cartridge shells with a flash composition. When cartridges prepared in this manner are ignited, it is found that the igniting flame is taken up by the coating of flash composition and spreads, enveloping the fuel in the shell, so as to produce more desirable burning characteristics without the need for deck loading or for double base fuel.

Usually the flash composition is most advantageously applied to the surface of the cartridge through the medium of a lacquer in which it is suspended or dissolved. Such a lacquer bearing flash composition may be conveniently sprayed into the cartridge shells to produce the desired coating. Other methods of coating flash composition onto the walls of the cartridge may also be employed as will be evident to those skilled in the art. For example, flash composition may be dusted onto the walls of the cartridges after they have been coated with a tacky material.

The benefits of the present invention are obtained in general to the extent that the coating covers the inside surface of each cartridge shell. Preferably, however, at least 75% of the inside surface area is coated, and even more preferably the inside surface is substantially completely coated, although satisfactory results may be obtained in some cases with less extensive coatings.

Numerous flash compositions may be used. In general, it is found that relatively slow burning flash compositions are more desirable. Flash compositions of the type taught in Young Patent No. 1,935,495 have been found particularly desirable. As is more fully set forth in that patent, such flash compositions comprise an intimate admixture of a nitro-aromatic compound and an oxidizing agent. Suitable nitro-aromatic compounds are trinitrotoluene, tetrinitroaniline,

tetryl, hexanitrodiphenylamine, picric acid, tri-nitroresorcinol, and related compounds. Among the useful oxidizing agents may be mentioned the chromates or dichromates of sodium, potassium, ammonium, barium, and lead, the nitrates of barium, potassium, and lead, and the peroxides of barium and lead. Usually it is preferred to employ an oxidizing agent of minimum hygroscopicity, as potassium dichromate. Among other flash materials which may be employed may be mentioned black powder grains and smokeless powder grains. Mixtures of different flash compositions also may be employed.

If the flash compositions are to be applied in lacquer form, any suitable lacquer and solvent compatible with the composition may be used. Nitrocellulose in acetone, for example, is desirable for use with tetryl-potassium dichromate mixtures. Nitrocellulose in ether-alcohol mixtures may be successfully used with black powder.

Large sized slow burning particles of fuel are often desirable for use in propellant fuel cartridges, such as, for example, those used for starting engines. In order to successfully employ such difficultly ignitable and easily extinguishable large particles of fuel, complicated deck loading, using charges of smaller sized fuel, has usually been necessary. It has been found, however, that cartridges of the present invention, having inside shell coatings of fuel igniting flash composition, may consist of single or straight charges of one large size of fuel particles only.

For example, cylindrical particles of colloided nitrocellulose fuel, as large or larger than .240" diameter by .260" long, may be used in this manner with entirely satisfactory results.

The invention, however, may also be used to advantage in cartridges containing smaller fuel particles.

A specific embodiment of the invention will be described in connection with the drawing which shows a longitudinal section through a starter cartridge of the present invention.

The cartridge comprises a cylindrical laminated paper shell 11, about 3 $\frac{3}{8}$ " long and about 1" in diameter, with a metal ferrule 13 crimped thereon. Ferrule 13 has an opening 15 in its center. Insulating disk 17 lies against ferrule 13 and contains a hole registering with the hole 15 in ferrule 13. Next to disk 17 and spanning registering hole 15 in ferrule 13 and insulating disk 17 lies metal terminal 19. Insulating disk 21 covers metal terminal 19 and disk 17. Metal ferrule 13 is electrically connected to electric match head igniter 27 by match terminal 23. Terminal 19 also extends to electric matchhead igniter 27. Igniter 27 is of the type described in Pratt Patent No. 2,309,978. On the walls of shell 11 lies flash composition 29.

Flash composition 29 was prepared and applied in the following manner. Nine and one-half ounces of scrap nitrocellulose film were dissolved in one gallon of acetone. To 240 cc. of the lacquer so produced were added 300 g. of a finely divided admixture composed of 75% tetryl and 25% potassium dichromate. The resulting suspension was sprayed into shell 11, coating substantially the entire interior, where it was permitted to dry. Enough lacquer suspension was sprayed in the shell to supply about 1.5 grams of dry inflammable film containing the tetryl-potassium dichromate mixture.

Shell 11 was then loaded with 22 g. of rela-

tively coarse grains of single base colloided nitrocellulose powder, generally represented at 31 in the drawing. This powder was in the form of cylindrical pellets, about 0.325 in. in length and about 0.313 in. in diameter. Following loading, the cartridge was closed by crimping in cellulose nitrate wad 33 and was ready for use in the conventional manner by placing it in operative relation with a starter device and igniting it by connecting it by means of ferrule 13 and terminal 19 to a suitable source of electric current. The cartridge prepared as above described was found to produce consistently satisfactory performance. Also, cartridges prepared in this manner were found to be highly resistant to quenching when used in succession in a single piece of apparatus.

Cartridges of the present invention may, of course, be modified in many ways without departing from the present invention. For example, the cartridge shells and other parts may be made of different materials than those described. Also, the end wads may be coated with flash composition as well as the rest of the interior of the cartridge shell. Other flash compositions and lacquers may be employed as is outlined above.

Also other sizes and compositions of fuel may be employed. For example, the invention may be used to improve the action of deck loaded cartridges and cartridges containing double base powder. Furthermore, different igniting means than the electric match head mentioned above can be used. For example, deflagrating compositions in various forms, such as globules, tubes, fuse heads, and coated wads ignited by spark gaps, bridge wires or percussion caps may be employed with the present invention.

The invention will be found to be generally applicable wherever it is desired to produce a propellant fuel cartridge having improved igniting characteristics.

What is claimed is:

1. A propellant fuel cartridge comprising an elongated shell, a coating of flash composition on the inside surface of said shell, an igniting means positioned to ignite said coating, and a fuel comprising single base nitrocellulose granules, said coating having an area of at least substantially 75% of the side surface of the shell so as to produce a flame for the envelopment of the fuel upon actuation of the igniting means.

2. A propellant fuel cartridge according to claim 1 in which the flash composition comprises an intimate admixture of a nitro-aromatic compound and a compound selected from the group consisting of chromates and dichromates.

ALVIN M. COHAN.

#### REFERENCES CITED

The following references are of record in the file of this patent:

#### UNITED STATES PATENTS

| Number    | Name    | Date          |
|-----------|---------|---------------|
| 2,096,698 | Lowy    | Oct. 19, 1937 |
| 2,299,466 | Coffman | Oct. 20, 1942 |
| 2,207,936 | Nardone | July 16, 1940 |
| 2,362,927 | Pratt   | Nov. 14, 1944 |

#### FOREIGN PATENTS

| Number | Country       | Date |
|--------|---------------|------|
| 27,343 | Great Britain | 1909 |